

# UNITED STATES PATENT OFFICE.

PASQUALE ZAPPI, OF YOUNGSTOWN, OHIO, ASSIGNOR OF ONE-FOURTH TO JOSEPH J. SPOTTS, OF YOUNGSTOWN, OHIO.

## FIREPROOF COMPOSITION.

Specification of Letters Patent.

Patented Jan. 2, 1917.

1,211,028.

No Drawing.

Application filed May 23, 1916. Serial No. 99,464.

To all whom it may concern:

Be it known that I, PASQUALE ZAPPI, a subject of the King of Italy, and resident of Youngstown, county of Mahoning, and State of Ohio, have invented certain new and useful Improvements in Fireproof Compositions, of which the following is a specification.

This invention relates broadly to a fire-proof composition, and more particularly to a fireproof insulation material.

The primary object of the invention is to provide an incombustible composition capable of being molded to form slabs, bricks or blocks for use in building construction, and which is adapted to be used in slab form as a substitute for lath and plaster, as a protective lining for safes and vaults, and as an insulation covering or lagging for boilers, steam pipes and the like.

A further object is to provide a composition of the character mentioned which will not crack, craze, or scale off after being heated, which is a non-conductor of sound, heat and electricity, which is light in weight, and which may be sawed and nailed in the manner of wood.

A further object within the contemplation of the invention is to provide a composition which, used as an interior finish in building construction, is perfectly sanitary and affords no harbor in which insects may find lodgment.

The composition consists of certain materials or ingredients mixed together, preferably in about the following proportions, by volume.

|                |    |           |    |
|----------------|----|-----------|----|
| Gypsum         | 44 | per cent. |    |
| Sawdust        | 30 | "         | 40 |
| Asbestos fiber | 20 | "         |    |
| Kaolin         | 5  | "         |    |
| Boric acid     | 1  | "         |    |

Slight variations in the proportions may be resorted to without changing the general character of or materially affecting the efficiency of the composition.

To the above materials, dry mixed, sufficient water is added to reduce the whole to a plastic mass of the proper consistency for turning into molds or for applying in the desired manner. As is obvious, the material may be handled commercially in its dry state and then reduced to a plastic form only when ready to use.

What is claimed is—

1. A plastic composition comprising thirty parts of a vegetable fibrous material, forty-four parts gypsum, twenty parts asbestos fiber, five parts kaolin and one part boric acid.

2. A non-conductive plastic composition consisting of the following ingredients mixed in about the proportions named:

|                |    |           |    |
|----------------|----|-----------|----|
| Gypsum         | 44 | per cent. | 65 |
| Sawdust        | 30 | "         |    |
| Asbestos fiber | 20 | "         |    |
| Kaolin         | 5  | "         |    |
| Boric acid     | 1  | "         | 70 |

In testimony whereof, I affix my signature in presence of two subscribing witnesses.

PASQUALE ZAPPI.

Witnesses:

JAMES F. FANAGHER,  
GEO. SWANSTON.